

## UNITED STATES PATENT OFFICE.

EDWIN M. BAKER, OF ANN ARBOR, MICHIGAN, ASSIGNOR TO CHRISTIAN GIRL, OF KALAMAZOO, MICHIGAN.

## PROCESS OF AND MEANS FOR NICKEL PLATING.

No Drawing.

Application filed January 5, 1923. Serial No. 610,927.

To all whom it may concern:

Be it known that I, EDWIN M. BAKER, a citizen of the United States, residing at Ann Arbor, in the county of Washtenaw and State of Michigan, have invented a certain new and useful Improvement in Processes of and Means for Nickel Plating, of which the following is a full, clear, and exact description.

10 This invention relates to a process of and means for electro-plating, and more particularly to the application to articles, such as spring bars or plates, a hard, dense and finely-divided crystalline deposit of nickel, which deposit will adhere firmly to the plates or other articles to which it is applied and which will withstand all of the ordinary incidents of use, including a buffing operation, without being readily cut or worn away 20 thereby. A further object of the invention is to accomplish the electro-plating of articles at a speed greatly in excess of that which has been obtainable heretofore. Other and more limited objects of the invention will appear 25 hereinafter, and will be realized in and through the steps and combinations thereof embodied in the claims forming part hereof.

In the practice of my process, as used for the nickel-plating of steel bars or plates, 30 such as are employed in the manufacture of vehicle springs and bumpers, the plates are first thoroughly cleaned in any approved manner, as by a polishing treatment; and then immersed in a special, heated nickel-plating bath having special nickel electrodes, through which electric current is passed under a very high amperage as compared with that which has been in standard use heretofore for electro-plating purposes. After 35 this nickel-plating treatment, the plates are copper plated in a vigorously-agitated bath having a temperature of approximately 30° C. using current under a high density, as before. After the copper-plating operation, 40 the bars or plates need not be buffed, but may then be given a final nickel-plating treatment, in a bath of the same character and under substantially the same conditions as employed in the first nickel-plating operation.

For the nickel-plating bath, I prepare a solution in which the following ingredients

are employed, in about the proportions stated, for each gallon of solution:

|                                                                       |    |
|-----------------------------------------------------------------------|----|
| 32 oz. nickel sulphate ( $\text{NiSO}_4 \cdot 7\text{H}_2\text{O}$ )  | 55 |
| 3.3 oz. nickel chloride ( $\text{NiCl}_2 \cdot 6\text{H}_2\text{O}$ ) |    |
| 2 oz. boric acid ( $\text{H}_3\text{BO}_3$ )                          |    |

While the proportions stated may be varied somewhat, with comparable results, those given are best adapted for successful results. The solution is heated (as by means of a steam coil) to a temperature of from 65° C. to 90° C., the best results having been obtained hitherto by employing a temperature of about 85° C. For the anodes, I employ substantially pure nickel (at least 99% pure). In order to obtain this purity it is preferable to employ, and I do employ, electrolytic nickel, although any form of very pure nickel (over 99%) would give satisfactory results.

With a bath constituted and heated in the manner described, and employing such pure nickel anodes, I preferably employ, for the plating work, current at a density of approximately 100 amperes per square foot of metal treated, as distinguished from the ordinary practice wherein a current density of 3 to 7 amperes per square foot is employed. However, many good results may be secured by using a current density of approximately 50 amperes per square foot of metal treated. As a result, the plates or bars will be provided with a hard, dense, and finely-divided crystalline deposit of nickel, which adheres firmly to the bars or plates and which is not readily cut or rubbed through, as by friction in ordinary use or in buffing.

After the initial nickel-treating operation, the bars or plates are placed in a copper plating bath, the bath containing the following ingredients, preferably in about the proportions stated, per gallon of solution:

|                                                                         |    |
|-------------------------------------------------------------------------|----|
| 28 oz. of copper sulphate ( $\text{CuSO}_4 \cdot 5\text{H}_2\text{O}$ ) | 95 |
| 11 oz. of sulphuric acid ( $\text{H}_2\text{SO}_4$ )                    |    |

The copper-plating solution is used at a temperature of preferably 30° C., employing approximately the same electric current density as is the case in the nickel plating operation. In order to secure an effective copper-plating at this current density, it is necessary that the solution be vigorously agitated, and this agitation is accomplished

by means of air, which may be introduced below the surface of the bath in any approved manner, as by means of an air supply pipe having perforations therethrough. 5 While the proportions hereinbefore set forth for the copper sulphate and the sulphuric acid per gallon of solution are those which are preferred, a considerable latitude in such proportions is permissible. For instance, 10 the copper sulphate may vary from 25 to 35 oz. per gallon and the sulphuric acid from 3 to 12 oz. per gallon, without materially changing the nature of the copper-plating. Furthermore, a fairly satisfactory result as 15 to plating may be obtained under a wide variation of current density—from 2 or 3 amperes to 200 amperes per square foot. However, the plating secured at the low current density will be quite soft and the time 20 consumed in such operation will be excessive. The temperature also may be varied from 20° C. to about 50° C. with very satisfactory results. However, the best results are obtained by using the proportions of bath-in- 25 gredients, the temperature, and the current density set forth hereinbefore. By so doing, a hard, dense and adhesive coating is secured, the operation requires but a very short time as compared with that required 30 in ordinary copper-plating practice and produces a much smoother coating than is obtained in ordinary practice, usually rendering unnecessary a buffering operation prior to the final nickel-plating operation. 35 After the copper-plating treatment, the bars or plates may be buffed to insure a smooth surface for the final-nickel coating. This final coating is applied in the same manner as the first coating or plating. After 40 the final nickel-plating operation, the bars or plates may be buffed.

The practical advantages of the process herein described are that I am enabled greatly to improve the character of the coating applied to the bars or plates and to effect a great reduction in the time required for effecting such coating. The coating is made up of a hard, dense, and very-finely divided crystalline deposit of nickel which adheres 45 firmly to the articles coated and which withstands, to a marked degree, buffering operations and the ordinary incidents of use. The coating is much harder than that which is secured by ordinary nickel plating operations, 50 and this hardness and density enhance the wear-and-rust-resistant qualities of the coating. Another and very important advantage of my process is that I am enabled to reduce the time for completely plating the 55 plates or bars to about one-thirtieth that which is ordinarily required for this purpose.

The employment of a heated bath with high current-density enables me to plate with great rapidity and to employ for this

purpose substantially pure nickel for the anodes. The use of such nickel results in a deposit of substantially pure nickel upon the cathodes and in maintaining the bath substantially free from sludge. The presence 70 of a chloride or chlorides in the bath facilitates both the speed of the plating-operation and the quality of the nickel deposit.

Also, by the employment of a chloride in the bath, the time required for the plating operation is greatly shortened and, if nickel chloride be used as well as nickel sulphate, the bath will be substantially free from all metal or ammonium salts and will contain practically no other salts than those of nickel. 75

Having thus described my invention, 80 what I claim is:

1. The process of nickel-plating articles which comprises the following steps:

(a) Subjecting the articles to an electro-plating treatment, employing therein anodes of substantially pure nickel, a current density of approximately 100 amperes per square foot of metal treated, and a bath heated to about 85° C. and containing the following ingredients, in substantially the proportions stated, per gallon of solution:

32 oz. nickel sulphate ( $\text{NiSO}_4 \cdot 7\text{H}_2\text{O}$ )

3.3 oz. nickel chloride ( $\text{NiCl}_2 \cdot 6\text{H}_2\text{O}$ )

2 oz. boric acid ( $\text{H}_3\text{BO}_3$ ).

(b) Subjecting the said articles to a copper-plating treatment in a bath agitated with air and at a temperature of approximately 30° C., said bath containing the following ingredients in approximately the proportions stated per gallon:

28 oz. of copper sulphate ( $\text{CuSO}_4 \cdot 5\text{H}_2\text{O}$ )

11 oz. of sulphuric acid ( $\text{H}_2\text{SO}_4$ ).

(c) Nickel-plating the articles in substantially the same manner and in a bath of the same character as set forth in step (a) hereinbefore.

2. The process of nickel-plating articles which comprises the following steps:

(a) Subjecting the articles to an electro-plating treatment, employing therein anodes of substantially pure nickel, a current density not materially less than 50 amperes per square foot of metal treated, and a heated bath containing the following ingredients, in substantially the proportions stated, per gallon of solution:

32 oz. nickel sulphate ( $\text{NiSO}_4 \cdot 7\text{H}_2\text{O}$ )

3.3 oz. nickel chloride ( $\text{NiCl}_2 \cdot 6\text{H}_2\text{O}$ )

2 oz. boric acid ( $\text{H}_3\text{BO}_3$ ).

(b) Subjecting the said articles to a copper-plating treatment in an agitated bath containing the following ingredients, in approximately the proportions stated, per gallon:

28 oz. copper sulphate ( $\text{CuSO}_4 \cdot 5\text{H}_2\text{O}$ )

11 oz. sulphuric acid ( $\text{H}_2\text{SO}_4$ ).

(c) Nickel-plating the articles in substantially the same manner and in a bath of

the same character as employed in the former nickel-plating operation.

3. The process of nickel-plating articles which comprises the following steps:

5 (a) Nickel-plating the articles in a heated bath, employing therewith substantially pure nickel anodes and a current density not materially less than 50 amperes per square foot of metal treated;

10 (b) Copper-plating the articles in a suitable bath under high current density, with the agitation of such bath;

(c) Nickel-plating the articles thus treated in substantially the same manner as employed for the first operation.

4. The process of nickel-plating articles which comprises the following steps:

(a) Nickel-plating the articles in a heated bath, employing therewith substantially pure nickel anodes and a current density of not materially less than 50 amperes per square foot of metal treated;

(b) Copper-plating the articles in a suitable bath;

25 (c) Nickel-plating the articles thus treated in substantially the same manner as employed for the first operation.

5. The process of nickel-plating articles which comprises the following steps:

30 (a) Nickel-plating the articles in a heated solution of nickel sulphate, nickel chloride, and boric acid, with the employment of an electric current of high density;

(b) Copper-plating the articles in a solution of copper sulphate and sulphuric acid, subjected to agitation, and with the employment of an electric current of high density;

40 (c) Subjecting the copper-plated articles to a nickel-plating operation similar to that employed for the first operation.

6. The process of nickel-plating articles which comprises the following steps:

(a) Nickel-plating the articles in a heated bath and with the employment of substantially pure nickel anodes and an electric current of high density;

(b) Copper-plating the articles in a bath subjected to agitation and with the employment of an electric current of high density;

50 (c) Subjecting the copper-plated articles to a nickel-plating operation similar to that first described.

7. The process of nickel-plating articles which comprises the following steps:

(a) Nickel-plating the articles in a heated bath containing a chloride in solution and with the employment of substantially pure nickel for the anode or anodes and an electric current of high density.

(b) Copper plating the articles in a bath subjected to agitation and with the employment of an electric current of high density.

60 (c) Nickel-plating the copper-plated article.

8. The process of nickel-plating articles which comprises the following steps:

(a) Nickel-plating the articles in a heated bath containing nickel chloride in solution and with the employment of substantially 70 pure nickel for the anode or anodes and an electric current of high density.

(b) Copper-plating the articles in a bath subjected to agitation and with the employment of an electric current of high density. 75

(c) Subjecting the copper-plated articles to a nickel-plating operation preferably similar to that employed for the first operation.

9. The process of nickel-plating articles 80 which comprises the following steps:

(a) Nickel-plating the articles in a heated bath containing a chloride and with the employment of substantially pure nickel for the anode or anodes and an electric current of 85 high density.

(b) Copper-plating the articles in a bath subjected to agitation by air under pressure introduced below the surface of the bath and with the employment of an electric current 90 of high density.

(c) Nickel-plating the articles thus copper-plated and preferably by means of a nickel-plating operation similar to that employed for the first operation. 95

10. The process of nickel-plating articles which comprises the following steps:

(a) Nickel-plating the articles.

(b) Copper-plating the articles thus nickel plated. 100

(c) Nickel-plating the articles in a heated bath containing nickel chloride in solution and with the employment of substantially pure nickel for the anode or anodes and an electric current of high density. 105

11. The process of nickel-plating articles which comprises the following steps:

(a) Nickel-plating the articles.

(b) Copper-plating the articles in a bath subjected to agitation and with the employment of electric current of high density. 110

(c) Nickel-plating the articles in a heated bath containing nickel chloride in solution and with the employment of substantially pure nickel for the anode or anodes and an electric current of high density. 115

12. The process of nickel-plating articles which comprises the following steps:

(a) Nickel-plating the articles.

(b) Copper-plating the articles in a bath 120 subjected to agitation by air under pressure introduced below the surface of the bath and with the employment of an electric current of high density.

(c) Nickel-plating the articles thus copper-plated. 125

In testimony whereof, I hereunto affix my signature.

EDWIN M. BAKER.